# EUROPEAN PATENT SPECIFICATION

(11) **EP 2 479 299 B1**
(45) Date of publication and mention of the grant of the patent: **29.05.2013**
(21) Application number: 11151788.4
(22) Date of filing: 24.01.2011
(51) Int. Cl.: C22C 9/00, H01B 1/02

(54) **Copper tubular cable for power lines**
Rohrförmiges Kupferkabel für Leistungsleitungen
Câble tubulaire en cuivre pour lignes d'alimentation

(43) Date of publication of application: 25.07.2012
(73) Proprietor: La Farga Lacambra, S.A., 08509 Les Masies de Voltrega (ES)
(72) Inventor: Guixà Arderiu, Oriol, 08509, LES MASIES DE VOLTREGA (ES); Garcia Zamora, Miquel, 08509, LES MASIES DE VOLTREGA (ES); Ferrer Crusellas, Nuria, 08509, LES MASIES DE VOLTREGA (ES); Riera Fontana, Lluis, 08509, LES MASIES DE VOLTREGA (ES)
(74) Representative: Isern-Jara, Nuria

(56) References cited:
- EP-A2- 0 569 036
- EP-A2- 0 702 375
- US-A1- 2005 161 129

## Description

### Descriptive Memory

Copper tubular cable for overhead power lines known as CATC (Copper Alloy Tubular Conductor).

### Object of the invention

The present invention relates to a cable formed by a poly-microalloyed copper tube of small diameter, from 6 to 15 mm, and wall thickness varying between 0.8 and 1.5 mm, which is used as the basis on which to braid one or several levels of poly-microalloyed copper wire of a diameter preferably between 1 and 2.5 mm.

### Background of the invention

In the field of transport and distribution of electricity by means of overhead lines, high-capacity aluminium steel (ACSR) cables are well known. The electricity industry is in constant growth due to the soaring energy demand. The problems that currently exist within the sector of overhead power lines can be summarized in the following points:
1.- The loss of mechanical properties of the Aluminium steel high-capacity cables (ACSR) in situations where there is high seasonal demand for power (mainly located in large cities or coastal areas), which leads to blackouts, drops in voltage, etc.
2.- The social rejection to the installation of new high-voltage power line paths, the complex environmental impact studies that this entails and the complex administrative procedures that have to be followed result in the need to search for better as well as efficacious, alternatives, such as the repowering by replacement of existing conductors with high temperature, low-sag conductors (HTLS).

The increase in current airline capacity, either transient or permanent, maintaining the existing configuration and the conductor section, necessarily involves a significant increase in the operating temperature of the conductors by the Joule effect. Nominal operating conditions of a conductor cable ensure a service life which fluctuates between 20 and 30 years. Nonetheless, these occurrences of temporary overload on the lines cause the cables to exceed the limit operating temperature and during prolonged periods this decreases the service life of the cable.

Both the decrease in the service life of the conductor as well as the low transport capacity are factors that lead companies to consider changing the conventional conductors for others that support greater power transmission capacity at high temperatures. For example, JP 51117121 discloses an alloy for overhead electric power lines consisting of (by wt.%) 0.5-1.0% Si, 0.1-0.5% Ag and additionally 0.05 - 0.5% of at least one element selected from B and rare earth, rest Cu. The existence of a need to repower overhead lines optimally and efficiently, while reaching solutions for the conflicting parameters, has encouraged providers to focus their innovation activity on seeking for new high-capacity conductors, also considering that the metals used in the construction of the overhead lines should have three main features:
- low electrical resistance and as a result low losses due to the Joule effect.
- high mechanical resistance, i.e. offer high resistance to permanent or accidental stresses.
- Reasonable cost, because the remaining infrastructure on a transmission line is based on the conductor.

One of the main existing issues holding back the repowering of lines by the companies responsible for power transmission is the high economic cost involved in carrying out the modifications. Currently, repowering the lines with the aim of preventing the loss of mechanical and electrical properties is carried out by increasing the section of the high-capacity cables, which involves an increase in the weight of the cable and, consequently, an increase in the weight that the towers have to withstand. This normally involves replacing the high-voltage tower for another that is able to withstand the weight, which involves an increase in the cost of the investment.

### Description of the invention

The copper tubular cable for overhead power lines known as CATC (Copper Alloy Tubular Conductor) object of the present registration, resolves the aforementioned drawbacks, providing, in addition, other additional advantages which will be evident from the description provided hereinafter.

The invention consists in the formation of a cable of characterist geometry defined by a poly-microalloyed copper tube of small diameter, from 6 to 15 mm and a wall thickness varying between 0.8 and 1.5 mm, which is used as the basis on which to braid a plurality of poly-microalloyed copper strands of a diameter preferably between 1 and 2.5 mm, in one or several levels.

Alloying the tube and the strands that conform it consist of adding multiple chemical elements in concentrations ranging between 0.000 and 0.231 % of atomic weight to the high-purity copper. Said chemical elements include:
- a group of metal elements formed by Zn, Pb, Sn, Ni, Mn and Ag;
- a group of semi-metal or metalloid elements formed by Sb, Se and As; and
- Oxygen;

More specifically, each one of the aforementioned essential elements is found within the concentration ranges, in % of atomic weight, shown in the following Table I.

As for the electrical properties, it is a well-known fact that the conductors that operate on an alternate current exhibit the skin effect. The skin effect on a conductor is calculated as: ${δ}^{2} * \left({e}^{- {/}_{δ} α}-1\right) + δ * α$

Where:
- δ: is the penetration of the electromagnetic field in the material under study; for copper its value is 9.5 mm
- α: Thickness of the conductor

According to the above, it is shown that the lower the value of α, the more the effective conductivity of the cable will approach the DC conductivity which is the highest obtainable; and the sections being equal, a tubular cable covered with a crown of strands, has a smaller thickness α than a solid cable.

Thus, the novel geometric configuration of the copper tubular cable for overhead power lines (CATC) together with the composition of the elements that conform it, give it several characteristics that resolve the drawbacks of the main conductors known according to the current state of the art, including:
- Improved conductivity.
- Increase in the torsional resistance, preventing it from turning on itself when faced with accumulations of snow or ice.
- Formation of an interior space that allows coolants (gaseous or liquid) to circulate through the tube.
- Formation of an interior space that allows for the installation of optical fibres and/or other light elements acting as information transmitters ; and/or allows for the installation of a steel strand that improves the tensile strength of the line.
- Reduction of the wind pressure on the cable

To complete the description and in order to help better understand its characteristics, accompanying the descriptive memory herein is a set of drawings in whose figures, by way of illustration and in a non-limiting manner, the most significant details of the invention are represented.

### Brief description of the drawings

Figure 1.- Perspective view of the tubular cable for CATC power lines according to the present invention.
Figure 2.- Shows a comparison between the increases in temperature during the flow of current of an LA-180 cable and a CATC-95 cable (data at an ambient temperature of 40ºC).
Figure 3.- Shows a comparison of the properties of an ACSR-type cable with a CATC-type cable in accordance with the present invention which shows the feasibility of replacing a conventional aluminium ACSR-type conductor for the CATC conductor.

### Description of a preferred embodiment

In view of ***the described figures*** and according to the numbering adopted, a preferred, although non-limiting, embodiment of the invention can be observed ***therein**,* which consists of an annular conductor section defined by a tube (1) with an exterior diameter D1 and an interior diameter D2 that is used as the basis on which to braid one or several levels of poly-microalloyed copper wires of diameter D3 (2). The conductor thus conformed has an empty cylindrical space of diameter D2 along its entire length.

The CATC cable according to the present invention is characterized by having values of Mechanical Resistance (Rm) between 400-600 MPa, an annealing temperature greater than 340ºC, an emissivity coefficient of 0.72 and an electrical conductivity of 90-98 IACS.

As shown in Fig. 2, because the aluminium exhibits greater yield strength than copper, on increasing the intensity, the CATC cable can continue operating to substantially higher temperatures.

On the other hand, comparing the physical and electrical characteristics of the CATC cable with those of a conventional aluminium-steel (ACSR) cable, it is shown (Fig.3), for example, that the ACSR LA-280 cable can be replaced by a CATC-95 cable, transporting 34% more power at the maximum operating temperature and weighing 129 kg less per km.

In conclusion and in accordance with that set out in Figures 2 and 3, it is feasible to substitute an aluminium-type ACSR conductor for the tubular CATC conductor, which will provide:
- An increase in the transmission of power at peaks with operating temperatures sustained indefinitely at 150ºC and transiently (500 hrs) at 175 ºC of about 25% to 60%.
- No substantial increase in total linear weight
- No need for additional support cables that are not part of the cabling for spans of up to 350 m and greater distances in the case of including support.
- With a high emission factor that allows for greater heat removal and prevents overheating at high intensities

## Claims

1. Copper tubular cable for overhead power lines, of the type used for the transport of alternate or direct current, **characterized in that** the alloying of the exterior wires and the interior tube that define it, is a result of adding to the high-purity copper the following elements in concentrations that range in % of atomic weight between the following values:
- Zn: 0.002 - 0.010
- Pb: 0.009 - 0.021
- Sn: 0.016 - 0.161
- Ni: 0.005 - 0.043
- As: 0.001 - 0.002
- Sb: 0.001 - 0.005
- Ag: 0.002 - 0.012
- O: 0.040 - 0.119
- Mn: 0.000 - 0.231
- Se: 0.000 - 0.161

2. A copper tubular cable for overhead power lines, according to claim 1 **characterized in that** it is conformed by a poly-microalloyed copper tube of small diameter, from 6 to 15 mm, and a wall thickness preferably varying between 0.8 and 1.5 mm, which constitutes the basis on which to braid a plurality of poly-microalloyed copper strands of a diameter preferably between 1 and 2.5 mm, in one or several levels.

3. A copper tubular cable for overhead power lines, according to claim 2, **characterized in that** both the tube and the strands may be covered with insulation material.

4. A copper tubular cable for overhead power lines, according to the previous claims, **characterized in that** the interior tube generates an empty space that allows installation in its interior of optical fibres and/or other light elements that are transmitters of information, and/or a steel strand that improves the tensile strength of the line, and/or the circulation of coolant fluids (gaseous or liquid).

## Patentansprüche

1. Kupferrohrkabel für elektrische Hängeleitungen der Art, die für den Transport von Wechsel- oder Gleichstrom verwendet werden, **dadurch gekennzeichnet, dass** die Legierung der Außenkabel und des Innenrohrs, aus denen es gebildet wird, dadurch entsteht, dass man dem hochreinen Kupfer die nachstehend angegebenen Elemente in einem % beimengt, der jeweils zwischen den nachstehend angegebenen Werten in Atomgewichtsprozent liegt.
Zn: 0,002-0,010
Pb: 0,009-0,021
Sn: 0,016-0,161
Ni: 0,005-0,043
As: 0,001-0,002
Sb: 0,001-0,005
Ag: 0,002-0,012
O: 0,040-0,119
Mn: 0,000-0,231
Se: 0,000-0,161

2. Kupferrohrkabel für elektrische Hängeleitungen nach Anspruch 1, **dadurch gekennzeichnet, dass** es aus einem poly-mikrolegierten Kupferrohr mit geringem Durchmesser zwischen 6 und 15 mm und einer Wandstärke von bevorzugt 0,8 bis 1,5 mm gebildet wird, das die Grundlage für eine Reihe von ein- oder mehrlagig darauf geflochtenen poly-mikrolegierten Kupferkabeln mit einem Durchmesser von vorzugsweise 1 bis 2,5 mm bildet.

3. Kupferrohrkabel für elektrische Hängeleitungen nach Anspruch 2, **dadurch gekennzeichnet, dass** sowohl das Rohr wie auch die Kabel von einem Isoliermaterial überzogen sein können.

4. Kupferrohrkabel für elektrische Hängeleitungen nach den vorhergehenden Ansprüchen, **dadurch gekennzeichnet, dass** das Innenrohr einen Hohlraum bildet, das die Anordnung von optischen Fasern und/oder anderen Lichtelementen zur Übertragung von Information und/oder einem Stahlseil zur Erhöhung der Zugfestigkeit der Leitung und/oder von zirkulierenden Kühlfluiden (Gase oder Flüssigkeiten) in seinem Inneren ermöglicht.

## Revendications

1. Câble tubulaire en cuivre pour lignes électriques aériennes, du type utilisé pour le transport du courant électrique alternatif ou continu, **caractérisé en ce que** l'alliage des câbles extérieurs et du tube intérieur qui le définit est le résultat d'ajouter au cuivre de très grande pureté les éléments suivants à des concentrations qui varient en % de poids atomique entre les valeurs suivantes :
Zn : 0,002-0,010
Pb : 0,009-0,021
Sn : 0,016-0,161
Ni : 0,005-0,043
As : 0,001-0,002
Sb : 0,001-0,005
Ag : 0,002-0,012
O : 0,040-0,1 19
Mn : 0,000-0,231
Se : 0,000-0,161 1

2. Câble tubulaire en cuivre pour lignes électriques aériennes, selon la revendication 1, **caractérisé en ce qu'**il est formé d'un tube en cuivre polymicroallié d'un petit diamètre, de 6 à 15 mm, et d'une épaisseur de paroi variable, de préférence entre 0,8 et 1,5 mm, qui constitue la base sur laquelle est effectué le torsadage d'une série de câbles en cuivre polymicroalliés, d'un diamètre compris de préférence entre 1 et 2,5 mm, sur une ou plusieurs des couches.

3. Câble tubulaire en cuivre pour lignes électriques aériennes, selon la revendication 2, **caractérisé en ce que** le tube comme les câbles peuvent être recouverts d'une matière isolante.

4. Câble tubulaire en cuivre pour lignes électriques aériennes, selon les revendications précédentes, **caractérisé en ce que** le tube intérieur génère un espace creux qui permet la mise en place, en son sein, de fibres optiques ou d'autres éléments de lumière qui sont des transmetteurs d'information, ou un câble en acier qui améliore la résistance à la traction de la ligne, ou la circulation de fluides réfrigérants (gazeux ou liquides).
